

## UNITED STATES PATENT OFFICE.

BERTRAND S. SUMMERS, OF PORT HURON, MICHIGAN.

## ART OF MAKING PAPER PULP.

No Drawing.

Application filed July 9, 1924. Serial No. 724,974.

My invention relates more particularly to an improvement in the so-called kraft process. This process is an alkaline process in which the material is subjected to a liquor containing primarily caustic soda and sulphide of soda. In the digestion of wood by this liquor, obnoxious odors arise due to mercaptans being formed which pollute the air surrounding the works. It is also a peculiarity of the kraft pulp that while it makes a very strong pliable paper it is brown in color and is very difficult to bleach and when bleached losses considerable of its characteristic qualities.

I have discovered that phosphoric acid and its compounds which are soluble in hot strong caustic liquor have the peculiar effect when added to the liquor of greatly lessening or obviating the odor arising from this process and of rendering the resultant pulp much more easily bleached. The pulp is usually stronger and more pliable. By my improved process I am able to produce a fully bleached pulp capable of being blended in high grade white sheets and at the same time preserving the valuable qualities of kraft pulp. I prefer to use an alkaline phosphate either the acid phosphate of sodium or the full metallic sodium phosphate as it is readily obtainable on the market at a reasonable price. A quarter of 1% of phosphoric acid by weight of the moist chips is sufficient to bring about these results. However, I do not confine myself to this proportion. The quality of the pulp may be changed by varying the relative proportion of the sulphur and phosphoric compounds in the liquor, the amount of phosphate to be used depending upon the paper which is to be made from the pulp produced.

I will now give an example of the commercial operation of my process. In a digester containing about 800 cubic feet of

liquor I introduce about 300 cubic feet of 45 white liquor running about 7 pounds of active alkali per cubic foot. To this I add about 500 cubic feet of black liquor from a previous cook and as the chips are being charged into the digester I usually sprinkle 50 from 50 to 100 pounds of phosphate figured as tri-sodic phosphate. I prefer to cook the batch from 2½ to 3 hours reaching a maximum temperature of 180° centigrade. Such an operation produces in the neighborhood of 3 tons of the soft pliable pulp capable of being bleached to full white. Instead of using tri-sodium phosphates other compounds containing phosphoric acid may be employed.

I claim:

1. A process of producing kraft pulp which consists in digesting the fiber in kraft liquor containing phosphoric acid compounds.

2. A process of producing kraft pulp which consists in digesting the fiber in kraft liquor containing a soluble phosphate.

3. A process of producing a kraft pulp which consists in subjecting vegetable material to the action of a solution containing a caustic alkali, a sulphate of an alkali metal and a phosphate.

4. A process for producing bleached kraft pulp which consists first in digesting the 75 vegetable material in a kraft liquor to which phosphoric acid or a salt thereof has been added and then subjecting the pulp to a bleaching operation substantially as described.

5. A process for making bleached kraft pulp which consists in cooking the material in a kraft liquor containing a soluble phosphate and then subjecting the resulting pulp to a bleaching operation substantially as described.

BERTRAND S. SUMMERS.